

## 1

3,065,177

## HIGH TEMPERATURE GREASES

Bruce W. Hotten, Orinda, Calif., assignor to California Research Corporation, San Francisco, Calif., a corporation of Delaware  
No Drawing. Filed Mar. 14, 1960, Ser. No. 14,514  
5 Claims. (Cl. 252—49.6)

This invention relates to lubricating greases. More particularly, it relates to lubricating oil compositions composed of an oil of lubricating viscosity thickened by a thickening agent to grease-like consistency, such greases being characterized by high melting points and wherein the thickening agent is nonmetallic.

This application is a continuation-in-part of Hotten patent application Serial No. 606,993, filed August 30, 1956, and now abandoned.

It is prevailing practice to use salts of certain fatty acids or other suitable acids and certain metals to produce high melting point greases. Thus, sodium and lithium stearates, also sodium and lithium salts of certain mono-amides of polycarboxylic acids are employed as thickeners to produce high melting point greases. Metal salt thickeners are disadvantageous, however, because the metals therein promote oxidation.

Although nonmetal-containing grease thickening agents have been proposed heretofore, most of these do not produce grease compositions having high dropping points (ASTM method D-566-42).

It is an object of the present invention to provide greases having high dropping points and in which the thickeners are of the nonmetallic type.

It is a particular object of the invention to provide greases having dropping points in the neighborhood of 400° F. or more, preferably 500° F. or more, and wherein the thickeners are nonmetallic.

Yet another object of the invention is to provide novel compounds which can be prepared economically, which are nonmetallic in nature and which are useful, among other things, as grease thickeners.

These and other objects of the invention will be apparent from the ensuing description and the appended claims.

In accordance with the present invention, it has been discovered that high melting grease compositions are obtained by incorporating in certain polysiloxane base oils of lubricating viscosity a thickening agent consisting of a mixture of diamides of terephthalic acid and a terephthalamic acid (or an ester thereof). Thus, high melting grease compositions are obtained by thickening certain polysiloxane oils of lubricating viscosity with the combination of terephthaldiamides and terephthalamic acids or esters thereof.

The terephthaldiamides are of the type exemplified by the formula



wherein the R's are alkyl radicals containing from 1 to 3 carbon atoms, and n is a number from 0 to 1.

Esters of terephthalamic acids which are contemplated

## 2

herein in combination with terephthaldiamides include those of the formula



wherein R represents hydrogen or the methyl or ethyl radicals, and R1 is an alkyl radical containing from 1 to 2 carbon atoms.

The preferred diamides of terephthalic acid are those having the type formula



The combination of terephthaldiamides and terephthalamic acids or their esters effectively thickens to grease consistency certain methyl, phenyl polysiloxanes. These oils are characterized as polymethylphenylsiloxanes having a medium methyl-phenyl ratio. As determined by the infrared analysis procedure described in "Naval Research Laboratory Report," P-2746 (1946), by Smith, French and O'Neil, the methylphenyl ratios are evaluated according to the peaks observed in the infrared analysis; these ratios have values from 0.3 to 0.5; that is, the methyl radicals and the phenyl radicals are present in the polymethylphenylsiloxane in proportions such that the ratio of methyl radicals to phenyl radicals has values from 0.3 to 0.5, based on infrared analysis.

The combination of terephthaldiamides and terephthalamic acids (or esters thereof) is used in amounts of 15%, by weight, to 50%, preferably 20% to 30%. The weight ratio of terephthaldiamides to terephthalamic acids (or esters thereof) is from 1:4 to 1:1.

The thickener combination of the invention may be incorporated in such base oils in varying amounts. Where a high dropping point is not important, the combination may be used in amounts as low as 5%, or less may be employed, but where high dropping points (i.e., about 500° F. or higher) are desired, larger amounts of thickener combination should be employed, for example, 10% or higher, all such percentages being by weight based on the finished grease. It is preferred to use no more than 30%. All percentages are by weight based on finished product.

The following specific examples will serve to illustrate the practice and advantages of the invention.

## EXAMPLE I

## 55 Mixture of N,N'-Di-p-Tolylterephthaldiamide and N-tolylterephthalamic Acid

1284 grams (12 mols) of p-toluidine and 582 grams (3 mols) of dimethyl terephthalate were heated and stirred together at 170-210° C. for 6 hours. The product was washed three times with boiling benzene and was dried. A yield of 733 grams was obtained consisting of one-half N,N'-di-p-tolylterephthaldiamide and one-half N-tolylterephthalamic acid having the following formulas:



and



The saponification number of the product was 154 and nitrogen content was 6.54%.

#### EXAMPLE II

A mixture of 25 grams of the product of Example I (one-half methyl-N-tolylterephthalamic acid and one-half *N,N'-di-p-tolylterephthaldiamide*) and 75 grams of a poly(phenylmethyl siloxane) oil (Dow Corning DC-550) was heated with stirring to 600° F.; pan cooled; then milled in a needle valve mill at 4000 p.s.i. The resulting smooth, soft grease had an ASTM dropping point of 500+° F.; worked penetration ( $P_{60}$ ) of 348; and a high speed bearing life of 510 hours (average of two runs, 354 and 665 hours) at 450° F. and of 307 hours (average of two runs, 212 and 401 hours) at 500° F. The high speed bearing life test (quoted as MIL-G-25013) was run as follows:

A 204K Conrad type 8-ball bearing packed with grease was operated at 10,000 r.p.m. continuously for 22 hours at the designated temperature. The bearing was then cooled to room temperature during a period of 2 hours, then run at 10,000 r.p.m. for another 22 hours. This cycle was repeated until the bearing failed.

Other greases containing thickener combinations of this invention are illustrated, together with test results, in Table I hereinbelow. The compositions were blended and treated by processes similar to those set forth in Example II hereinabove.

The base oil in each of the compositions A, B, C, D and E was a polymethylphenylsiloxane wherein the methyl-phenyl ratio had a value of 0.4 (based on infrared analysis). This base oil is further identified as DC 550, which is sold as such by Dow Corning Corporation, Midland, Michigan.

The base oil for composition F was a polymethylphenylsiloxane wherein the methyl-phenyl ratio had a value of 0.4. This base oil is further identified as Dow Corning QF-4039 fluid which is sold as such by the Dow Corning Corporation of Midland, Michigan.

TABLE I

| Composition                              | Amount,<br>Wt.<br>Percent | Appearance         | ASTM<br>Dropping<br>Point,<br>° F. | $P_{60}$ | Bearing<br>Life<br>(Hours) |
|------------------------------------------|---------------------------|--------------------|------------------------------------|----------|----------------------------|
| <b>A</b>                                 |                           |                    |                                    |          |                            |
| (a) Base Oil.....                        | 75                        | Liquid.....        |                                    |          |                            |
| (b) Terephthalyl-di-p-toluidide.....     | 25                        |                    |                                    |          |                            |
| <b>B</b>                                 |                           |                    |                                    |          |                            |
| (a) Base Oil.....                        | 75                        | do.....            |                                    |          |                            |
| (b) Methyl,N-p-tolylterephthalamate..... | 25                        |                    |                                    |          |                            |
| <b>C</b>                                 |                           |                    |                                    |          |                            |
| (a) Base Oil.....                        | 75                        | Smooth Grease..... | 494                                | 382      | 1 529                      |
| (b) Terephthalyl-di-p-toluidide.....     | 12.5                      |                    |                                    |          |                            |
| (c) Methyl,N-p-tolylterephthalamate..... | 12.5                      |                    |                                    |          |                            |
| <b>D</b>                                 |                           |                    |                                    |          |                            |
| (a) Base Oil.....                        | 75                        | do.....            | 500                                | 348      | 1 307                      |
| (b) Terephthalyl-di-p-toluidide.....     | 12.5                      |                    |                                    |          |                            |
| (c) N-p-tolylterephthalamic acid.....    | 12.5                      |                    |                                    |          |                            |
| <b>E</b>                                 |                           |                    |                                    |          |                            |
| (a) Base Oil.....                        | 75                        | do.....            |                                    | 367      |                            |
| (b) Terephthalyl-di-p-toluidide.....     | 18.75                     |                    |                                    |          |                            |
| (c) N-tolylterephthalamic acid.....      | 6.25                      |                    |                                    |          |                            |
| <b>F</b>                                 |                           |                    |                                    |          |                            |
| (a) Base oil.....                        | 75                        | do.....            |                                    | 404      |                            |
| (b) Terephthalyl-di-p-toluidide.....     | 12.5                      |                    |                                    |          |                            |
| (c) N-p-tolylterephthalamic acid.....    | 12.5                      |                    |                                    |          |                            |

<sup>1</sup> Average of 2 runs.

It will, therefore, be apparent that nonmetallic grease thickeners described herein form greases which are characterized by high dropping points and, in many cases by exceptionally high dropping points. The latter characteristic is highly advantageous in view of the fact that the thickeners are nonmetallic.

Such greases may include other ingredients, such as oxidation and/or corrosion inhibitors, etc.

I claim:

1. A grease composition comprising a major proportion of a polysiloxane base oil of lubricating viscosity and, in an amount sufficient to thicken said oil to the consistency of a grease, the combination of a terephthaldiamide having the type formula



wherein the R's are alkyl radicals containing from 1 to 3 carbon atoms, and n is a number from 0 to 1, and a compound of the formula



wherein R is selected from the group consisting of hydrogen and alkyl radicals containing from 1 to 2 carbon atoms, and R1 is an alkyl radical containing from 1 to 2 carbon atoms, wherein said polysiloxane is a polymethylphenylsiloxane wherein the methyl-phenyl ratio has values from 0.3 to 0.5, and the weight ratio of terephthaldiamide to said compound is from 1:4 to 1:1.

2. A grease composition consisting essentially of a polymethylphenylsiloxane base oil and, from 15% to 50%, by weight, of the combination of a terephthaldiamide of the formula



wherein the R's are alkyl radicals containing from 1 to 3

5

carbon atoms, and  $n$  is a number from 0 to 1, and a compound of the formula



wherein R is selected from the group consisting of hydrogen and alkyl radicals containing from 1 to 2 carbon atoms, and R<sub>1</sub> is an alkyl radical containing from 1 to 2 carbon atoms, wherein the methyl-phenyl ratio of said polysiloxane has values from 0.3 to 0.5, and wherein the weight ratio of said terephthaldiamide to said compound is from 1:4 to about 1:1.

3. A grease composition consisting essentially of a polymethylphenylsiloxane base oil, and from 20% to 30%, by weight, of the combination of a terephthaldiamide of the formula



wherein the R's are alkyl radicals containing from 1 to 3

6

carbon atoms, and  $n$  is a number from 0 to 1, and a compound of the formula



wherein R is selected from the group consisting of hydrogen and alkyl radicals containing from 1 to 2 carbon atoms, and R<sub>1</sub> is an alkyl radical containing from 1 to 2 carbon atoms, wherein the methyl-phenyl ratio of said polysiloxane has values from 0.3 to 0.5, and wherein the weight ratio of said terephthaldiamide to said compound is from 1:4 to about 1:1.

20 4. A grease composition comprising a major proportion of a polymethylphenylsiloxane base oil, and from 20% to 30%, by weight, of the combination of a terephthaldiamide of N,N'-di-p-tolylterephthaldiamide and N-tolylterephthalamic acid, wherein the terephthaldiamide-terephthalamic acid weight ratio is from 1:4 to 1:1.

5. A grease composition comprising a major proportion of a polymethylphenylsiloxane base oil, and from 20% to 30%, by weight, of the combination of equal parts, by weight, of N,N'-di-p-tolylterephthaldiamide and N-tolylterephthalamic acid, wherein the methyl-phenyl ratio of said polymethylphenylsiloxane has values from 0.3 to 0.5.

References Cited in the file of this patent

35 UNITED STATES PATENTS

2,710,839 Swakon et al. \_\_\_\_\_ June 14, 1955  
2,808,427 Hotten \_\_\_\_\_ Oct. 1, 1957